

# UNITED STATES PATENT OFFICE.

ALBERT WESTLAKE AND PAUL POETSCHKE, OF NEW YORK, N. Y.; SAID POETSCHKE  
ASSIGNOR TO SAID WESTLAKE.

## MANUFACTURE OF FIBROUS CAPS FOR BOTTLES AND OTHER CONTAINERS.

1,160,478.

Specification of Letters Patent.

Patented Nov. 16, 1915.

No Drawing.

Application filed December 12, 1913. Serial No. 806,307.

To all whom it may concern:

Be it known that we, ALBERT WESTLAKE and PAUL POETSCHKE, both citizens of the United States, and residents of the city, county, and State of New York, have invented certain new and useful Improvements in the Manufacture of Fibrous Caps for Bottles and other Containers, of which the following is a specification.

10 Our invention relates to that class of caps, seals or closures for bottles, jars, storage, and other containers, such caps, seals and closures being composed essentially of fibrous material of vegetable or

15 animal origin, and their equivalents.

Our object is to secure a fibrous material which, by its nature, cannot discolor or present a cutting edge and which will be sufficiently durable for purposes of transportation, delivery and temporary storage, can be easily destroyed after use, or after removal from bottle or container, can be temporarily replaced to preserve the remainder of the bottle or container contents, 25 a feature vitally necessary to the protection of the contents of the container from extraneous contamination during temporary storage and use of the contents.

The object of our invention is to impart 30 certain characteristics to such fibrous material which will render it more sanitary, cleanly, less absorbent, and sufficiently resistant to the liquids, or other food products contained in the bottle, jar or container, 35 not affecting them in a deleterious manner as regards appearance, odor, or wholesomeness, and which is adapted, when properly applied, to make a more perfect fabrication of the material, comprising the cap or seal, 40 thereby providing closer contact with the bottle, jar or other container than has heretofore been the case with non-metallic contrivances, thereby producing a practically air-tight and effective seal or closure.

45 Our invention is more particularly designed for sealing glass or porcelain bottles or containers, used for milk or drinking water, for daily distribution and consumption, which articles being especially liable 50 to contamination in transit or handling, and of vital importance to the health of the community, are required to be protected by efficient sanitary measures. This improved fiber cap or sanative seal may be used for

various other liquids, pickles, preserves, jellies, foods, drugs or medicines that require cheap and effective and hygienic sealing.

We have found that ordinary fiber paper cannot be shaped over the mouth of a bottle or container and made to hold a definite position or shape without mechanical means of retention. Ordinary paper is either tough or stiff, has surface imperfections and springs away after being mechanically shaped, even when applied with the aid of heat or moisture, so as to facilitate adaptation to the various forms or construction of the mouth of the bottle or other container. We have found this to be the case even after dipping the paper or fibrous material in melted paraffin, or other waxy or gummy substances, or by supplying an inner seal of wax paper, paraffin, or similar preparations. We have therefore devised the hereinafter described process which results in a fibrous material having sufficient plasticity and flowing or molding properties under the application of heat, combined with the property of setting rigidly and promptly upon cooling to ordinary temperatures; thus insuring an absolute contact with the container to which it is applied and adapting itself to all interstices of the bottle or other container, yielding a cap or closure or seal which, when thus applied, is impervious to moisture, is non-absorbent, insoluble in water or other liquids usually contained in the bottle to which it is applied, and will maintain its sealing qualities and guard the contents against exposure or contamination.

It is also sufficiently strong, tenacious and durable to resist displacement, or tearing during transit or handling, also to resist thermal changes, such as extreme cold and heat of winter and summer, or exposure to direct rays of the sun. To accomplish these results, we begin with a suitable fiber of vegetable or animal origin,—for instance, cellular pulp prepared by chemical or mechanical means from such fibers. This pulp, before it is converted into sheets suitable for the purpose, is, preferably, treated while in this state by any of the methods that will allow the sheet, irrespective of thickness, to remain in a soft and pliable condition, similar to filter or blotting paper. This pulp may also be treated with the various sizing or

water-proofing agents, applied in the paper industry to insure resistance to water, provided all soluble deleterious substances are eliminated so that they do not enter the finished paper.

In order further to promote softness in the finished fibrous material, an emulsion prepared from certain aliphatic resins or mixtures of aliphatic resins with conifer resins, or their equivalents, by treatment with a solution of a base, such as sodium hydroxid, or its equivalent, may be incorporated with the pulp, the mass being subsequently treated with alum or other suitable precipitating agent. For example, the following emulsion may be used:—

|                  |       |
|------------------|-------|
| Water            | 78.5% |
| Colophony        | 10.0% |
| Shellac          | 10.0% |
| Sodium carbonate | 1.5%  |

Excessive hot calendering and undue pressure is avoided in forming the sheets or strips in order to bring out a material of 25 loosely-felted fibers, further fabrication or condensation of this paper being reserved for its heating and shaping process on the bottle, jar or other container. This fiber, when made of selected widths, according to 30 the demand for resistance of the bottle contents, is passed over rolls in a continuous manner, and thereby coated or impregnated, and, if desired, separate layers may be united thereby so as to produce the desired 35 ply and thickness. The coating material is preferably composed of certain aliphatic and conifer resins or their equivalents, either alone or in admixture. These substances may also be mixed with certain harmless 40 mineral fillers, such as silica or calcium sulfate. For example, the following combination may be used:—

|                        |     |
|------------------------|-----|
| White turpentine resin | 25% |
| Colophony              | 15% |
| Shellac                | 25% |
| Calcium sulfate        | 35% |

The proportions and character of the ingredients must be varied so as to secure a 50 fluid of the correct viscosity and consistency for coating when moderate heat is applied to the mixture, or various solvents such as ethyl alcohol may be incorporated therewith so as to obtain the proper consist-

ency of the material at still lower temperature.

The mixture of aliphatic and conifer resins, with or without mineral fillers, may also be applied by pulverizing the mass and sifting this onto the paper, previously warmed by passing over heated rolls, or after previously moistening the paper with a suitable solvent. The coated paper is then printed and stamped out into round disks of suitable size, the operation being continuous with the coating process; for instance, for the size of the so-called standard quart or pint milk bottle of the present date, the disk should be three and three-quarter inches in diameter. The result of this process is a fibrous disk of the required thickness, which is practically insoluble in water, thoroughly innocuous, sanitary, rigid, and tenacious at normal temperatures, and capable of becoming plastic and moldable at elevated temperatures.

By the above described treatment we have succeeded in preparing a fibrous material which, when used for caps and other seals or closures for bottles, jars, and other containers, possesses those hygienic and commercial qualities which have been found necessary and advantageous.

We claim:

1. Process of manufacturing fibrous caps for bottles and other containers which comprises the treating of fibrous material when in a soft and pliable condition with an emulsion prepared from aliphatic resins by treatment with sodium hydroxid or equivalent base and subsequently treating the mass with alum or equivalent precipitating agent.

2. A fibrous cap for bottles and other containers which is composed of fibrous material which has been rendered practically insoluble in water, innocuous, sanitary, rigid and tenacious at normal temperatures and capable of becoming plastic and moldable at elevated temperatures by the incorporation therewith while in a soft and pliable condition, of resinous substances, a sodium base and a precipitating agent substantially as described.

ALBERT WESTLAKE.  
PAUL POETSCHKE.

Witnesses:

LILLIAN MACKREHORST,  
W. P. PREBLE.